

## UNITED STATES PATENT OFFICE

TRUMAN S. FULLER AND DAVID BASCH, OF SCHENECTADY, NEW YORK, ASSIGNEES TO  
GENERAL ELECTRIC COMPANY, A CORPORATION OF NEW YORK

## ALUMINUM ALLOY

No Drawing.

Application filed December 13, 1923. Serial No. 680,516.

Our present invention comprises an improved cast alloy of aluminum, zinc and magnesium, and it is the object of our invention to improve the physical properties of the cast alloy.

Heretofore cast aluminum alloys containing copper have been improved by heat treatment. The improvement has been ascribed to the tendency of certain components, particularly copper-aluminum particles, to be thrown out of solution from the aluminum during the slow cooling after the heat treatment.

We have now discovered that aluminum alloy castings containing at least about 6% zinc and at least about 1/2% magnesium, but containing no substantial amount of copper, other than as a possible impurity, can be materially improved in mechanical properties by a heat treatment schedule which is hereinafter described in detail. The improvement due to heat treatment is especially marked in the case of aluminum alloys containing both zinc and magnesium and an even more marked improvement due to heat treatment is obtained when other alloying elements such as iron are present.

The improvement in mechanical properties due to heat treatment in an alloy of aluminum, magnesium and zinc, illustrates the benefits of our invention. A cast alloy comprising about 92.75 parts aluminum, about 6 parts zinc and about 1.25 parts magnesium, and excluding copper except as a negligible impurity has a tensile strength of about 26,000 pounds per square inch and a hardness of about 75 Brinell. When this alloy is heated to about 515° C. for about twenty-four hours, then is quenched in boiling water, and finally is aged either artificially at about 150° C. for three hours or more, or naturally the tensile strength is increased to about 35,000 pounds per square inch and the hardness is raised to about 104 Brinell.

Fuller Patent 1,273,762 of July 23, 1918, covers an aluminum alloy containing zinc, magnesium and iron, or various described equivalents. In accordance with this patent the cast alloy is mechanically worked, as by forging, rolling, or drawing. We have dis-

covered that the physical properties of the alloy may be improved without mechanical working by subjecting this cast alloy to a schedule of heat treatment.

For example, a cast aluminum alloy which has an approximate composition of aluminum 90.75%, zinc about 6%, iron 2%, and magnesium 1.25%, has without heat treatment a tensile strength of about 30,000 pounds and a hardness of 65 Brinell.

In accordance with our invention this cast alloy is given the following heat treatment: The alloy first is heated to a temperature of about 450 to 575° C. for about 24 hours and then is quenched, preferably in boiling water. Next the alloy is subjected to an aging treatment, for example, by heating to a temperature of about 150° C. for about one to three hours or more. Thereafter it may be allowed to cool naturally. As a result of this heat treating schedule the properties of the cast alloy are materially improved. The tensile strength is increased to 50,000 pounds and the hardness is raised to 115 Brinell.

In place of iron, or in addition to iron, other alloying metals, including silicon, may be added to the alloy of aluminum, magnesium and zinc.

In this specification and in the claims, the terms quenching and aging are intended to cover not only the specific temperatures enumerated herein but also the known variations of these temperatures which are permissible under various conditions. For example, it is known that aging of an alloy can be carried out at a lower temperature if the length of the aging step is correspondingly increased.

What we claim as new and desire to secure by Letters Patent of the United States, is—

1. The method of improving the tensile strength and hardness of an aluminum alloy containing at least about six per cent zinc, about one-half to two and one-half per cent of magnesium and about one to three per cent of iron, which consists in subjecting said alloy to a heat treatment at about 450 to 575° C. for about 24 hours, quenching in water and then heating to about 150° C. for about one to three hours.

2. A heat-treated alloy of aluminum being substantially devoid of copper and containing about six per cent zinc, about one and one-quarter per cent magnesium and two per cent iron, said alloy having a tensile strength of about 50,000 pounds per square inch and a hardness of about 155 Brinell but having otherwise substantially the properties of cast metal.
- 10 3. The method of improving the tensile strength of a cast alloy which is substantially devoid of copper but contains more than 80% aluminum, at least about 6% zinc and at least about  $\frac{1}{2}\%$  magnesium, which consists in heating the alloy between  $450^{\circ}$  C. and  $575^{\circ}$  C., quenching the alloy and then aging it at a temperature of about  $150^{\circ}$  C.
- 15

In witness whereof, we have hereunto set our hands this 12th day of December, 1923.

20 TRUMAN S. FULLER.  
DAVID BASCH.